

# United States Patent

[11] 3,615,621

[72] Inventor **Robert W. Lamon**  
Rochester, N.Y.  
[21] Appl. No. **751,745**  
[22] Filed **Aug. 12, 1968**  
[45] Patented **Oct. 26, 1971**  
[73] Assignee **Eastman Kodak Company**  
Rochester, N.Y.

---

[54] **4-PYRIMIDINETHIONE COMPOUNDS AS FOG  
INHIBITORS**  
19 Claims, No Drawings

---

[52] U.S. Cl..... **96/109,**  
260/251  
[51] Int. Cl..... **G03c 1/34,**  
C07d 5/18  
[50] Field of Search..... **96/109;**  
260/251

[56] **References Cited**  
UNITED STATES PATENTS  
3,040,047 6/1962 Sirakawa..... 96/109 X  
FOREIGN PATENTS  
753,434 7/1956 Great Britain..... 96/109

*Primary Examiner—Norman G. Torchin  
Assistant Examiner—Richard E. Fichter  
Attorneys—W. H. J. Kline and William E. Neely*

---

**ABSTRACT:** 4-Pyrimidinethione compounds are prepared by reaction of acyl isothiocyanate-tertiary enamine adducts with primary amines or ammonia. They are useful photographic fog inhibitors.

## 4-PYRIMIDINETHIONE COMPOUNDS AS FOG INHIBITORS

The present invention relates to a process for preparing certain 4-pyrimidinethione compounds and to their use as fog inhibitors in photography.

During development of a silver halide emulsion, small amounts of silver halide are reduced to metallic silver regardless of whether or not they have been exposed. This reduction of silver ion produces a background fog which is more specifically referred to as chemical fog.

Chemical fog, apparent in most silver halide systems, has been reduced by prior art methods of processing exposed silver halide material in the presence of compounds which restrict development of unexposed silver halide. Such compounds can be incorporated in the silver halide emulsion or in the processing solutions for developing such silver halide emulsions. Compounds which have been found to have a chemical fog inhibiting effect on emulsions which have been subjected to high temperature and high humidity conditions are referred to as emulsion stabilizers. On the other hand, compounds which have been found to have chemical fog inhibiting effects on emulsions which have not been exposed to adverse storage conditions are referred to as antifogants. Although a large number of emulsion stabilizers and antifogants have been used in the prior art, many of these compounds cause undesirable losses in emulsion speed and contrast and others lack adequate compatibility with emulsion gelatin.

It has now been found that fog reduction can be achieved by incorporating a small amount of certain 4-pyrimidinethiones in light-sensitive silver halide emulsions. The present invention includes a process for the production of certain 4-pyrimidinethiones, light-sensitive silver halide emulsions containing a 4-pyrimidinethione compound described hereinafter as an antifogant and a photographic element comprising a support having coated thereon a light-sensitive silver halide emulsion layer containing a 4-pyrimidinethione compound described hereinafter as an antifogant.

The 4-pyrimidinethione compounds utilized as antifogants in accordance with the present invention have the formula:

I



wherein R represents hydrogen or the organic portion of a primary organic amine, R<sub>1</sub> represents an alkyl group, an aralkyl group, e.g., benzyl or phenethyl, or a benzene nucleus, R<sub>2</sub> represents hydrogen, lower alkyl, lower alkoxy, carb(lower alkoxy) or a benzene nucleus, R<sub>3</sub> represents hydrogen or lower alkyl, and wherein R<sub>2</sub> and R<sub>3</sub> collectively represent a polymethylene chain having at least two carbon atoms, such as ethylene (-CH<sub>2</sub>CH<sub>2</sub>-), trimethylene (-CH<sub>2</sub>CH<sub>2</sub>CH<sub>2</sub>-), tetramethylene (-CH<sub>2</sub>CH<sub>2</sub>CH<sub>2</sub>CH<sub>2</sub>-), pentamethylene (-CH<sub>2</sub>CH<sub>2</sub>CH<sub>2</sub>CH<sub>2</sub>CH<sub>2</sub>-) or hexamethylene (-CH<sub>2</sub>CH<sub>2</sub>CH<sub>2</sub>CH<sub>2</sub>CH<sub>2</sub>CH<sub>2</sub>-), for example. When R<sub>1</sub> is a benzene nucleus, it is normally phenyl.

The term "lower alkyl" when used herein and in the claims, unless specifically indicated otherwise, refers to an alkyl group having one to six carbon atoms such as methyl, ethyl, propyl, isopropyl, butyl, isobutyl, pentyl or hexyl, for example.

The term "lower alkoxy" when used herein and in the claims, unless specifically indicated otherwise, refers to an alkoxy group having one to six carbon atoms such as methoxy, ethoxy, propoxy, isopropoxy, butoxy, isobutoxy, pentyloxy or hexyloxy, for example.

The term "a benzene nucleus" when used herein and in the claims, unless specifically indicated otherwise, refers to phen-

yl and substituted phenyl nuclei such as alkylphenyl, alkoxyphe- nyl, halophenyl or hydroxyphenyl nuclei, for example. Illustrative alkylphenyl nuclei include, for example, (o-,m-,p-)methylphenyl, (o-,m-,p-)ethylphenyl, (o-,m-,p-)propylphenyl, (o-,m-,p-)isopropylphenyl or (o-,m-,p-)butylphenyl. (o-,m-,p-)methoxyphenyl, (o-,m-,p-)ethoxyphenyl, (o-,m-,p-)propoxyphe- nyl, (o-,m-,p-)isopropoxyphe- nyl or (o-,m-,p-)butoxyphe- nyl, for example, are illustrative alkoxyphenyl nuclei. (o-,m-,p-)chlorophenyl, (o-,m-,p-)fluorophenyl or (o-,m-,p-)bromophenyl, for example, are illustrative halophenyl nuclei. (o-,m-,p-)hydroxyphenyl are illustrative of hydroxyphenyl nuclei.

Methoxycarbonyl, ethoxycarbonyl, propoxycarbonyl, isopropoxycarbonyl, butoxycarbonyl, pentyloxycarbonyl or hexyloxycarbonyl, for example, are illustrative of carb(lower alkoxy) groups.

The 4-pyrimidinethione compounds having the formula I are prepared in accordance with the process of the invention by reacting an acyl isothiocyanate-tertiary enamine adduct having the formula:

II



25

30

wherein R<sub>1</sub>, R<sub>2</sub> and R<sub>1</sub> have the meaning previously assigned to them and R<sub>a</sub> and R<sub>b</sub> each represents an alkyl group such as methyl, ethyl, propyl, isopropyl, butyl, isobutyl, pentyl, hexyl, octyl, decyl, etc., for example, especially a lower alkyl group having one to six carbon atoms and a benzene nucleus, and wherein



40

50

collectively represents a saturated 5 or 6 membered heterocyclic nucleus such as 1-pyrrolidinyl, piperidino, morpholino, 1-pyrazolidinyl or 3-oxazolidinyl, for example, with an amine having the formula R<sub>a</sub>NH<sub>2</sub> wherein R has the meaning previously assigned to it.

The adducts having the formula II are prepared by reacting a tertiary enamine having the formula:

III



55

60

wherein R<sub>a</sub>, R<sub>b</sub>, R<sub>2</sub> and R<sub>3</sub> have the meaning previously assigned to them with an acyl isothiocyanate having the formula:

IV



wherein R<sub>1</sub> has the meaning previously assigned to it.

Illustrative of the amines having the formula R<sub>a</sub>NH<sub>2</sub> are, for example, ammonia, alkylamines such as, for example, methylamine, ethylamine, propylamine, isopropylamine, butylamine, isobutylamine, pentylamine, hexylamine, heptylamine, octylamine, decylamine, dodecylamine, etc., hydroxyalkylamines such as, for example, 2-hydroxyethylamine, 3-hydroxypropylamine, 3-hydroxybutylamine, 4-hydroxybutylamine, 5-hydroxypentylamine, 6-hydroxyhexylamine, etc.; alkoxylalkylamines, such as, for example, 2-

methoxyethylamine, 2-ethoxyethylamine, 2-propoxymethylamine, 2-butoxyethylamine, 3-methoxypropylamine, 3-ethoxypropylamine, 3-propoxypropylamine, 4-methoxybutylamine, 4-ethoxybutylamine, etc., aralkylamines such as benzylamine or phenethylamine, for example, a carboxyalkylamine, such as, for example, carboxymethylamine, 2-carboxyethylamine, 3-carboxypropylamine, 4-carboxybutylamine, 5-carboxypentylamine, 6-carboxyhexylamine, etc., an  $\text{H}_2\text{N}-(\text{CH}_2)_n-\text{COOAlkyl}$  amine, wherein  $n$  represents a whole number from 1 to 4, such as, for example,



a dialkylaminoalkylamine such as, for example, 2-dimethylaminoethylamine, 2-diethylaminoethylamine, 2-dipropylaminoethylamine, 2-diisopropylaminoethylamine, 2-dibutylaminoethylamine, 3-dimethylaminopropylamine, 3-diethylaminopropylamine, 3-dipropylaminopropylamine, 3-diisopropylaminopropylamine, 4-dibutylaminopropylamine, 4-dimethylaminobutylamine, 4-diethylaminobutylamine, 4-dipropylaminobutylamine, 4-diisopropylaminobutylamine, 4-dibutylaminobutylamine, etc.; an arylamine, such as, for example, aniline (o-,m-,p-)toluidine, (o-,m-,p-)ethylaniline, (o-,m-,p-)anisidine, (o-,m-,p-)phenetidine, (o-,m-,p-)chloroaniline, (o-,m-,p-)bromoaniline, (o-,m-,p-)hydroxyaniline, 2,5-dimethoxyaniline, 2,5-diethoxyaniline, 1,2,3-xylidine, 1,2,4-xylidine, 1,3,2-xylidine, 1,3,4-xylidine, 1,4,2-xylidine, 1,3,5-xylidine, 4-aminodiphenyl, etc., and heterocyclic amines such as 4-(2-aminoethyl)morpholine



4-(aminopropyl)morpholine, 4-(aminobutyl)morpholine, 1-(2-aminoethyl)pyrrolidine, 1-(2-aminoethyl)-2-methyl-pyrrolidine or 1-(2aminoethyl)piperidine, for example.

As just noted, the adducts having the formula II are prepared by reacting a tertiary enamine having the formula III with an acyl isothiocyanate having the formula IV. The reaction is preferably carried out at room temperature, but the temperature may vary from about 10° C. to about 35° C. Advantageously, the reaction is carried out in an inert solvent in which the adducts are insoluble, such as, for example, dimethyl ether, diethyl ether, diisopropyl ether, p-dioxane, dimethoxyethane, benzene, etc., or chlorinated solvents, such as, for example, chloroform, dichloroethane, tetrachloroethane or carbon tetrachloride. A particular method of preparing tertiary enamine adducts is described by S. Hunig, K. Hubner and E. Benzig, in *Chem. Ber.* 95, 937-9 (1962).

The 4-pyrimidinethione compounds having the formula I are prepared by reacting an adduct having the formula II with an amine having the formula  $RNH_2$  wherein R has the meaning previously assigned to it. The reaction is normally carried out with agitation, such as stirring, in the presence of an inert solvent under basic reaction conditions. Suitable inert solvents include water and a lower alkanol such as, for example, ethanol, n-propyl alcohol or isopropyl alcohol. The reaction takes place without the necessity of heating and is preferably carried out at ambient conditions of temperature (i.e., about 10° C. to about 35° C.) and pressure, but an elevated temperature (e.g., above ambient temperature to about 100° C.) may be used to hasten the reaction. The basicity of the reaction mixture is advantageously maintained at a level, for example,

sufficient to preclude precipitation of intermediate reaction products before the reaction has an opportunity to proceed to the desired 4-pyrimidinethione product. In most cases the use of an excess of the amine compound having the formula  $\text{RNH}_2$ ,  
5 provides a sufficiently basic medium to solubilize intermediate reaction products through which reaction to the 4-pyrimidinethione product may proceed. In the event precipitation of any intermediate reaction product occurs, such intermediate product can be removed from the reaction mixture or can easily be converted to the 4-pyrimidinethione product by heating in the presence of a strong base, as is  
10 shown in the examples given hereinafter.

15 The preparation of the adducts having the formula II and the 4-pyrimidinethione compounds having the formula I is illustrated hereinafter. Temperatures in the examples and elsewhere herein are in degrees Centigrade unless otherwise indicated.

### Example 1

To a solution of 13.7 g. (0.10 mole) of 1-(N-pyrrolidino)cyclopentene in 70 ml. of dry diethyl ether was added dropwise, with cooling and stirring, 10.1 g. (0.10 mole) of acetyl isothiocyanate in 10 ml. of dry diethyl ether. After stirring in the cold for 2 hours, the orange precipitate which formed was collected, washed thoroughly with dry diethyl ether, then with 100 ml. of cold methanol, and finally with more dry diethyl ether. The resulting air-dried 1-(N-acetylthiocarbamoyl)-2-(N-pyrrolidino)-cyclopentene melted at 149°-150° C. dec. and weighed 20.0 g. Recrystallization from ethyl acetate to which was added a little methanol gave the analytical sample as orange prisms, m.p. 154°-155° C. dec. The infrared spectrum (KBr) showed maxima at  $3.15\mu$  (NH) and 5.95 (C=O). The N.M.R. spectrum agreed with the assigned structure in all respects.

The enamine product thus produced and identified as 1-(N-acetylthiocarbamoyl)-2-(N-pyrrolidino)-cyclopentene, 6.00 g. (0.025 mole), was suspended in 70 ml. of concentrated aqueous ammonia and the mixture was stirred until a solution 40 formed. Ethanol (30 ml.) was added portionwise to hasten solution. After standing overnight the solution was concentrated under vacuum and acidified to yield 3.72 g. of a tan colored solid, m.p. 234°-236° C. dec. Recrystallization from 45 methanol gave pale yellow needles of 6,7-dihydro-2-methyl-5 H-cyclopentapyrimidine-4(3H)-thione having an unchanged melting point.

### Example 2

50  $\beta$ -diethylaminostyrene was reacted with benzoyl isothiocyanate in accordance with the method described in example 1 for the preparation of the enamine adduct except that the reaction mixture was not cooled. During the course of the addition of the benzoyl isothiocyanate,  $\alpha$ -(N-benzoylthiocarbamoyl)- $\beta$ -diethylaminostyrene separated as a red oil which, as the mixture was stirred for several hours at room temperature, gradually solidified and granulated. The product was purified by precipitating from chloroform solution with ligroin (b.p. 35°-60°). Two repetitions of this process gave the analytical sample as red-orange prisms, m.p. 131°-132° C. dec. The infrared and N.M.R. spectra were consistent with the assigned structure.

The tertiary enamine adduct obtained as just described when reacted in equimolar amounts with cyclohexylamine and aqueous ethanol in a manner similar to that described in example 1 resulted in the precipitation of an intermediate product having the structure:



When the precipitated intermediate product was added to a 0.5N solution of sodium hydroxide in 50 percent aqueous ethanol and heated on a steam bath it cyclized to form 1-

cyclohexyl-2,5-diphenyl-4(1H)-pyrimidinethione having the formula:

VI



which, after recrystallization from ethanol melted at 215°-217° C.

## Example 3

To a stirred suspension of 2.00 g. (0.0073 mole) of the enamine adduct of example 1 in 20 ml. of ethanol was added 2 ml. of 2-aminoethanol. The resulting mixture was stirred for 2 hours during which time its color changed from orange to yellow. 6,7-Dihydro-1-(2-hydroxyethyl)-2-methyl-5H-cyclopentapyrimidine-4(1H)-thione precipitated as a solid, was collected, washed with ethanol and then air dried. Yield, 1.27 g., m.p. 240°-243° C. dec. Two recrystallizations from dimethylformamide gave the analytical sample as yellow plates, m.p. 243°-245° C. dec. 4

Three ml. of aniline were added to a suspension of 4.00 g. (0.0126 mole) of 1-(N-benzoylthiocarbamoyl)-2-(N-morpholino)cyclopentene in 35 ml. of ethanol. The resulting mixture was warmed briefly on a steam bath and stirred at room temperature for 30 minutes, or until all the red starting material was replaced by a yellow-orange solid product. The solid product was collected, washed with ethanol and air dried. 1-Anilino-2-(N-benzoylthiocarbamoyl)cyclopentane was thus obtained, weighing 3.77 g. and having a m.p. of 164° C. (transition). Two recrystallizations from chloroform-ethanol gave the analytical sample as fine yellow-orange needles, m.p. 168°-170° C. dec.

Four grams (0.0214 mole) of the product just obtained was suspended in a 0.5N solution of sodium hydroxide in 50 percent aqueous ethanol. The mixture was heated and swirled for 10 minutes on a steam bath then stirred for 1 hour at room temperature. 6,7-Dihydro-1,2-diphenyl-5H-cyclopentapyrimidine-4(1H)-thione precipitated as a yellow solid product, was collected, washed well with ethanol and air dried. Yield, 2.99 g., m.p. 230°-235° C. dec. Two recrystallizations from ethanol gave the analytical sample as yellow rods, m.p. 243°-245° C. dec.

Employing the general procedure of example 4 additional 6,7-dihydro-5H-cyclopentapyrimidine-4-thiones were prepared and are summarized in the following Table I.

TABLE I

6,7-dihydro-5H-cyclopentapyrimidine-4-thiones



| Example | R                                                                  | R1                            | Yield <sup>a</sup> , percent | M.P., ° C. | Recrystallization solvent |
|---------|--------------------------------------------------------------------|-------------------------------|------------------------------|------------|---------------------------|
| 5.....  | H                                                                  | C <sub>6</sub> H <sub>5</sub> | 79                           | b195-197   | Methanol.                 |
| 6.....  | CH <sub>3</sub>                                                    | C <sub>6</sub> H <sub>5</sub> | 76                           | b240-244   | Acetonitrile.             |
| 7.....  | CH <sub>2</sub> CH <sub>2</sub> OH                                 | C <sub>6</sub> H <sub>5</sub> | 80                           | b227-229   | Ethanol.                  |
| 8.....  | CH <sub>2</sub> CH <sub>2</sub> N(=O)C <sub>6</sub> H <sub>5</sub> | C <sub>6</sub> H <sub>5</sub> | 40                           | b200-201   | Ethanol.                  |
| 9.....  | CH <sub>3</sub>                                                    | CH <sub>3</sub>               | 77                           | b202-203   | Ethyl acetate.            |

<sup>a</sup> Yield based on crude material.

<sup>b</sup> Dec.

Additional 2,5-diphenyl-4(1H)-pyrimidinethiones listed in Table II hereinafter were prepared using the general procedure of example 2.

TABLE II

2,5-diphenyl-4(1H)-pyrimidinethiones



| Example | Yield <sup>a</sup> , percent                  | M.P., ° C. | Recrystallization solvent    |
|---------|-----------------------------------------------|------------|------------------------------|
| 10..... | CH <sub>2</sub> CH <sub>2</sub> OH            | 60         | b221-223 Chloroform-ethanol. |
| 11..... | CH <sub>3</sub>                               | 55         | b214-216 Chloroform-ethanol. |
| 12..... | CH <sub>2</sub> C <sub>6</sub> H <sub>5</sub> | 63         | b225-227 Acetonitrile.       |

<sup>a</sup> Yield based on crude material.

<sup>b</sup> Dec.

<sup>c</sup> Overall yield.

Certain enamine adducts obtained from the reaction of tertiary enamines and acyl isothiocyanates are unstable and yield on heating in ethanol a 4-oxazinethione. An example of such an enamine adduct is that resulting from the reaction of 1-(N-morpholino)cycloheptene and benzoyl isothiocyanate. In these cases the corresponding 4-pyrimidinethione compound can be obtained from the 4-oxazinethione compound as described hereinafter. The 4-pyrimidinethione compounds involved are those wherein R<sub>2</sub> and R<sub>3</sub> collectively represent tetramethylene or pentamethylene.

## Example 13

6,7,9,9-Tetrahydro-1-(2-hydroxyethyl)-2-phenyl-5H-cycloheptapyrimidine-4(1H)-thione

isothiocyanate, 16.3 g. (0.10 mole) was added dropwise, with stirring, to an ice cold solution of 18.1 g. (0.10 mole) 1-(N-morpholino)cycloheptene in dry ether. The mixture was kept cold for several hours and the orange solid which precipitated was collected by suction filtration. After washing thoroughly with ether, the solid, which became sticky on standing, was dissolved in 500 ml. of ethanol and the resulting solution filtered hot. Concentration of the filtrate to about 150 ml. and cooling gave the 4-oxazinethione intermediate product as orange needles. Yield 11.4 g. of 6,7,8,9-tetrahydro-2-phenyl-5H-cyclohepta-1,3-oxazine-4-thione, m.p. 170°-172° C. Two recrystallizations from ethanol gave the analytical sample as brilliant orange needles, m.p. 171°-173° C.;

$\lambda_{\text{max}}^{\text{CHCl}_3} = 292 \text{ m}\mu$

( $\epsilon$  2100), 341 ( $\epsilon$  13500). The infrared spectrum shows no NH or C = O bonds. The N.M.R. spectrum is consistent with 6,7,8,9-tetrahydro-2-phenyl-5H-cyclohepta-1,3-oxazine-4-thione.

Four grams (0.0155 mole) of the oxazine intermediate product obtained as just described was refluxed in a solution of 25 ml. of ethanol and 4 ml. of 2-aminoethanol until all the orange starting material was replaced by a bright yellow solid product (about 2 hours). Yield 4.04 g. of 6,7,8,9-tetrahydro-1-(2-hydroxyethyl)-2-phenyl-5H-cycloheptapyrimidine-4(1H)-thione, m.p. 226°-227° C. dec. Recrystallization from chloroform-ethanol gave tiny yellow needles of unchanged melting point.

Employing the general procedure of example 13 additional 6,7,8,9-tetrahydro-2-phenyl-5H-cycloheptapyrimidine-

4(1H)-thiones were prepared and are summarized hereinafter in Table III.

TABLE III

6,7,8,9-Tetrahydro-2-phenyl-5H-cycloheptapyrimidine-4(1H)-thiones



| Example | R                                               | Yield <sup>a</sup><br>percent | M.P., °C. | Recrystalliza-<br>tion solvent |
|---------|-------------------------------------------------|-------------------------------|-----------|--------------------------------|
| 14      | C <sub>6</sub> H <sub>5</sub>                   | 41                            | b263-265  | Chloroform-<br>ethanol.        |
| 15      | CH-CH <sub>3</sub><br>CH <sub>3</sub>           | 19                            | b207-209  | Ethanol.                       |
| 16      | CH <sub>3</sub> CH <sub>2</sub> CH <sub>2</sub> | 86                            | b212-213  | Ethanol.                       |
| 17      | H                                               | 96                            | b178-180  | Methanol.                      |
| 18      | CH <sub>2</sub> CH <sub>2</sub> N<br>O          | 49                            | b169-171  | Ethanol.                       |

<sup>a</sup> Crude material, based on 4-oxazinethione intermediate.

<sup>b</sup> Dec.

The conversion of 6,7,8,9-tetrahydro-2-phenyl-5-cycloheptoxazine-4-thione to 6,7,8,9-tetrahydro-2-phenyl-5H-cycloheptapyrimidine-4-thione compounds by refluxing with a primary amine in a solution of ethanol has been disclosed in examples 13-18.

However, it has been found that if 6,7,8,9-tetrahydro-2-phenyl-5H-cycloheptoxazine-4-thione is treated at room temperature with the primary organic amines, especially the more reactive primary organic amines, for example, alkylamines, the same products are obtained in improved yield. The use of hindered primary amines, such as isopropylamine or neopentylamine, for example, gives intermediate products which can be converted to the desired 4-pyrimidinethione products by treatment with an alkali. Preferably the alkali is employed in dilute form, such as, for example, 0.5 N alkali in 50 percent aqueous ethanol. When an alkali is needed the use of an appropriate dilute alkali will be readily apparent to one skilled in the art to which this invention is directed. The reaction scheme is illustrated hereinafter.



The corresponding oxazine containing a 6-membered fused ring (i.e., wherein R<sub>2</sub> and R<sub>3</sub> collectively represent tetramethylene) and which can be prepared as described by Hunig and Hubner (Chem. Ber. 95, pages 937-943, 1962), reacts similarly, as illustrated hereinafter. Certain compounds have been numbered for purposes of easy reference.



A mixture of aniline and (1) did not react appreciably although the mixture was maintained at room temperature for 24 hours. Reaction does occur when a mixture of aniline and (1) is refluxed together; 6,7,8,9-tetrahydro-1,2-diphenyl-5H-cycloheptapyrimidine-4(1H)-thione was so obtained.

#### Example 19

##### Preparation of 6,7,8,9-Tetrahydro-2-phenyl-1-propyl-5H-cycloheptapyrimidine-4-(1H)-thione

A mixture of 2.57 g. (0.01 mole) of 6,7,8,9-tetrahydro-2-phenyl-5H-cycloheptoxazine-4-thione having the formula 1 hereinbefore and 2 ml. of propylamine in 25 ml. of ethanol was stirred, without heating, for 1.25 hr. The yellow product was isolated by filtration, washed with fresh solvent and air-dried. Yield, 2.81 g., m.p. 212° dec. Recrystallization from ethanol gave pure product, m.p. 212°-213° dec.

35

#### Example 20

##### Preparation of 1-Hydroxy-2-(N-neopentylbenzimidoylthiocarbamoyl)-cycloheptene

A mixture of 2.57 g. (0.01 mole) of 6,7,8,9-tetrahydro-2-phenyl-5H-cycloheptoxazine-4-thione having the formula 1 hereinbefore and 2.6 ml. of neopentylamine in 20 ml. of ethanol was stirred, without heating, for 1.25 hours. The suspension which formed was filtered to give 2.14 g. of the adduct, 1-hydroxy-2-(N-neopentylbenzimidoylthiocarbamoyl)-cycloheptene



50 which after solution in dichloromethane and dilution with ligroin was recovered as a solid, m.p., 155°-156° dec.

#### Example 21

##### Preparation of 6,7,8,9-Tetrahydro-1-neopentyl-2-phenyl-5H-cycloheptapyrimidine-4(1H)-thione

One gram (0.00290 mole) of 1-hydroxy-2-(N-neopentylbenzimidoylthiocarbamoyl)-cycloheptene prepared as described in example 20, was warmed and swirled with 10 ml. of 0.5 N NaOH in 50 percent ethanol. The suspension which formed was stirred at room temperature for 1 hour, chilled, and filtered. After washing with aqueous ethanol the product weighed 0.88 g. (yield 93 percent), m.p. 218°-219° after softening and darkening at 209°-210°. Recrystallization from acetonitrile gave pure product melting at 221°-222° C. dec.

65 70 The identical material was also obtained by refluxing a mixture of 2.57 g. (0.01 mole) of 6,7,8,9-tetrahydro-2-phenyl-5H-cycloheptoxazine-4-thione and 2.6 ml. of neopentylamine in 20 ml. of ethanol for 4.5 hr. (56 percent yield).

The corresponding 4-pyrimidinethione compound wherein R<sub>2</sub> and R<sub>3</sub> collectively represent tetramethylene, i.e., 5,6,7,8-

75

tetrahydro-1-neopentyl-2-phenylquinazoline-4(1H)thione was similarly obtained by refluxing a mixture of 2.31 g. (0.01 mole) of 5,6,7,8-tetrahydro-2-phenylbenzoxazine-4(1H)-thione



and 2.6 ml. of neopentylamine in 20 ml. of ethanol for 3 hr. A yield of 95 percent was obtained. Upon recrystallization from acetonitrile the purified product melts at 216°-217.5°C.

Table IV hereinafter sets forth data with respect to various intermediates used in preparing the 4-pyrimidinethione antifogging compounds.

Table V hereinafter sets forth data with respect to 6,7-dihydro-5H-cyclopentapyrimidine-4-thione compounds. It supplements Table I.

TABLE IV

| Intermediate | Yield <sup>a</sup> (m.p. °C.) | Recrystallization solvent | Molecular formula | Calculated |     |      |      | Found |     |      |      |
|--------------|-------------------------------|---------------------------|-------------------|------------|-----|------|------|-------|-----|------|------|
|              |                               |                           |                   | C          | H   | N    | S    | C     | H   | N    | S    |
|              | 84%                           | Ethyl acetate/methanol    | C12H18N2OS        | 60.5       | 7.6 | 11.8 | 13.5 | 60.6  | 7.6 | 12.0 | 13.3 |
|              | 52% (131-132)                 | Chloroform/methanol       | C20H22N2OS        | 71.0       | 6.6 | 8.3  | 9.5  | 70.8  | 6.7 | 8.2  | 9.3  |
|              | 92% (168-170 dec.)            | Chloroform/methanol       | C19H18N2OS        | 70.8       | 5.6 | 8.7  | 9.9  | 70.5  | 5.8 | 8.6  | 9.8  |
|              | 85% (165-166 dec.)            | do                        | C22H24N2OS        | 72.5       | 6.6 | 7.7  | 8.8  | 72.4  | 6.7 | 7.5  | 8.8  |
|              | 44% (171-173 dec.)            | Ethanol                   | C15H15NOS         | 70.0       | 5.9 | 5.4  | 12.4 | 69.9  | 5.5 | 5.3  | 12.4 |

<sup>a</sup> Yields based on crude material.

TABLE V

| Example: | Yield, <sup>a</sup> percent | Molecular formula | Calculated |     |      |      | Found |     |      |      | $\lambda_{max.}^b$ | E-10 <sup>-3</sup> |
|----------|-----------------------------|-------------------|------------|-----|------|------|-------|-----|------|------|--------------------|--------------------|
|          |                             |                   | C          | H   | N    | S    | C     | H   | N    | S    |                    |                    |
| 1.....   | 89                          | C8H10N2S          | 57.8       | 6.1 | 16.9 | 19.3 | 57.6  | 6.1 | 16.8 | 19.4 | 290                | 9.4                |
| 3.....   | 72                          | C10H14N2OS        | 57.1       | 6.7 | 13.3 | 15.2 | 57.3  | 6.6 | 13.6 | 15.0 | 338                | 10.6               |
| 4.....   | 674                         | C19H16N2S         | 75.0       | 5.3 | 9.2  | 10.5 | 74.8  | 5.0 | 8.9  | 10.7 | 343                | 25.2               |
| 5.....   | 79                          | C12H12N2S         | 68.4       | 5.3 | 12.3 | 14.1 | 68.4  | 5.4 | 12.1 | 14.0 | 263                | 10.6               |
| 6.....   | 76                          | C14H14N2S         | 69.4       | 5.8 | 11.6 | 13.2 | 69.2  | 5.8 | 11.4 | 13.4 | 345                | 19.0               |
| 7.....   | 80                          | C15H16N2OS        | 66.2       | 5.9 | 10.3 | 11.8 | 66.0  | 5.9 | 10.5 | 12.0 | 308                | 19.4               |
| 8.....   | 40                          | C19H23N3OS        | 66.8       | 6.8 | 12.3 | 9.4  | 66.7  | 6.9 | 12.0 | 9.1  | 369                | 12.4               |
| 9.....   | 77                          | C9H12N2S          | 60.0       | 6.7 | 15.6 | 17.8 | 60.6  | 6.6 | 15.6 | 18.0 | 343                | 5.5                |
|          |                             |                   |            |     |      |      |       |     |      |      | 343                | 19.9               |
|          |                             |                   |            |     |      |      |       |     |      |      | 246                | 9.7                |
|          |                             |                   |            |     |      |      |       |     |      |      | 342                | 24.4               |
|          |                             |                   |            |     |      |      |       |     |      |      | 246                | 10.3               |
|          |                             |                   |            |     |      |      |       |     |      |      | 343                | 24.3               |
|          |                             |                   |            |     |      |      |       |     |      |      | 239                | 6.9                |
|          |                             |                   |            |     |      |      |       |     |      |      | 339                | 23.7               |

<sup>a</sup> Yield based on crude material.

<sup>b</sup> Overall yield.

<sup>c</sup> Determined in ethanol unless otherwise indicated.

<sup>d</sup> Determined in chloroform.

<sup>e</sup> Determined in dimethylformamide.

Table VI hereinafter sets forth data with respect to 2,5-diphenyl-4(1H)-pyrimidinethione compounds.

TABLE VI

| Yield, <sup>a</sup><br>percent | Molecular<br>formula                                             | Calculated |     |      |      | Found |     |     |      | $\lambda_{\text{max.}}^{\text{c}}$ | $E \cdot 10^{-3}$ |
|--------------------------------|------------------------------------------------------------------|------------|-----|------|------|-------|-----|-----|------|------------------------------------|-------------------|
|                                |                                                                  | C          | H   | N    | S    | C     | N   | H   | S    |                                    |                   |
| <b>Example:</b>                |                                                                  |            |     |      |      |       |     |     |      |                                    |                   |
| 2.....                         | <sup>a</sup> 69 C <sub>22</sub> H <sub>22</sub> N <sub>2</sub> S | 76.3       | 6.4 | 8.1  | 9.3  | 76.0  | 6.5 | 8.1 | 9.2  | 354                                | 19.8              |
| 10.....                        | 60 C <sub>18</sub> H <sub>16</sub> N <sub>2</sub> OS             | 70.1       | 5.2 | 9.1  | 10.4 | 69.9  | 5.5 | 9.1 | 10.3 | 243                                | 16.0              |
| 11.....                        | 55 C <sub>17</sub> H <sub>14</sub> N <sub>2</sub> S              | 73.4       | 5.1 | 10.9 | 11.5 | 73.4  | 5.0 | 9.9 | 11.5 | 348                                | 18.3              |
| 12.....                        | <sup>b</sup> 63 C <sub>23</sub> H <sub>18</sub> N <sub>2</sub> S | 77.9       | 5.2 | 7.9  | 9.0  | 77.7  | 5.2 | 7.8 | 8.9  | 351                                | 16.9              |
|                                |                                                                  |            |     |      |      |       |     |     |      | 354                                | 18.3              |

<sup>a</sup> Yield based on crude material.<sup>b</sup> Overall yield.<sup>c</sup> Determined in chloroform, except for second compound which was determined in ethanol.

Table VII hereinafter sets forth data with respect to 6,7,8,9-tetrahydro-2-phenyl-5H-cycloheptapyrimidine-4(1H)-thione compounds.

While dilute NaOH was the alkali actually employed wherein treatment with a dilute alkali is involved herein it will be understood that the other alkalies such as potassium

TABLE VII

| Yield, <sup>a</sup><br>percent | Molecular<br>formula                                 | Calculated |     |      |      | Found |     |      |      | $\lambda_{\text{max.}}^{\text{c}}$ | $E \cdot 10^{-3}$ |
|--------------------------------|------------------------------------------------------|------------|-----|------|------|-------|-----|------|------|------------------------------------|-------------------|
|                                |                                                      | C          | H   | N    | S    | C     | H   | N    | S    |                                    |                   |
| <b>Example:</b>                |                                                      |            |     |      |      |       |     |      |      |                                    |                   |
| 13.....                        | 86 C <sub>17</sub> H <sub>20</sub> N <sub>2</sub> OS | 68.0       | 6.1 | 9.3  | 10.7 | 67.8  | 7.0 | 9.1  | 10.9 | <sup>b</sup> 353                   | 18.0              |
| 14.....                        | 41 C <sub>21</sub> H <sub>20</sub> N <sub>2</sub> S  | 75.9       | 6.1 | 8.4  | 9.7  | 75.8  | 6.0 | 8.2  | 9.8  | <sup>b</sup> 362                   | 23.0              |
| 15.....                        | 19 C <sub>18</sub> H <sub>22</sub> N <sub>2</sub> S  | 72.5       | 7.4 | 9.4  | 10.7 | 72.3  | 7.5 | 9.2  | 10.5 | <sup>c</sup> 245                   | 8.5               |
| 16.....                        | 86 C <sub>18</sub> H <sub>22</sub> N <sub>2</sub> S  | 72.5       | 7.4 | 9.4  | 10.7 | 72.3  | 7.6 | 9.2  | 10.5 | <sup>c</sup> 347                   | 18.5              |
|                                |                                                      |            |     |      |      |       |     |      |      | 243                                | 9.4               |
| 17.....                        | 96 C <sub>15</sub> H <sub>16</sub> N <sub>2</sub> S  | 70.3       | 6.3 | 10.9 | 12.5 | 70.5  | 6.5 | 10.8 | 12.7 | <sup>c</sup> 347                   | 20.9              |
|                                |                                                      |            |     |      |      |       |     |      |      | 243                                | 16.3              |
| 18.....                        | 49 C <sub>21</sub> H <sub>27</sub> N <sub>3</sub> OS | 68.3       | 7.4 | 11.4 | 8.7  | 68.0  | 7.6 | 11.7 | 8.7  | <sup>c</sup> 253                   | 15.9              |
|                                |                                                      |            |     |      |      |       |     |      |      | 308                                | 12.7              |
|                                |                                                      |            |     |      |      |       |     |      |      | <sup>c</sup> 365                   | 6.0               |
|                                |                                                      |            |     |      |      |       |     |      |      | 245                                | 9.5               |
|                                |                                                      |            |     |      |      |       |     |      |      | <sup>c</sup> 348                   | 17.7              |

<sup>a</sup> Crude material, based on 4-oxazinethione intermediate.<sup>b</sup> Determined in chloroform.<sup>c</sup> Determined in ethanol.

Table VIII hereinafter lists various 4(1H)-pyrimidinethione compounds prepared in accordance with the present invention. These compounds were prepared by reacting the appropriate primary organic amine with the oxazine compound corresponding to the desired 4(1H)-pyrimidinethione. In the case of the unhindered amines the reactions were carried out at room temperature. Refluxing was employed in the case of hindered amines.

Table IX hereinafter sets forth data with respect to various intermediate compounds which can be cyclized, as shown hereinbefore, by treatment with dilute alkali, for example, to obtain 4(1H)-pyrimidinethione compounds containing a phenyl group attached to the carbon atom in the 2-position.

Table X hereinafter sets forth data with respect to the 4(1H) compounds containing a phenyl group attached to the carbon atom in the 2-position prepared by cyclization of the

40 hydroxide and lithium hydroxide, for example, can be similarly employed.

Other compounds that can be prepared in accordance with the invention include 5,6,7,8-tetrahydro-1,2-diphenylquinazoline-4(1H)-thione, 6,7-dihydro-1-n-butyl-2-methyl-5H-cyclopentapyrimidine-4-thione, 6,7-dihydro-1-n-butyl-2-phenyl-5H-cyclopentapyrimidine-4-thione, 1-ethyl-2,5-diphenyl-4(1H)-pyrimidinethione, 1-n-butyl-2,5-diphenyl-4(1H)-pyrimidinethione, 1- $\gamma$ -hydroxypropyl-2,5-diphenyl-4(1H)-pyrimidinethione, 6,7,8,9-tetrahydro-1-methyl-2-phenyl-5H-cycloheptapyrimidine-4(1H)-thione, 6,7,8,9-tetrahydro-1-n-butyl-2-phenyl-5H-cycloheptapyrimidine-4(1H)-thione, 5,6,7,8-tetrahydro-1-methyl-2-phenylquinazoline-4(1H)-thione and 5,6,7,8-tetrahydro-1-n-butyl-2-phenylquinazoline-4(1H)-thione, for example.

TABLE VIII



| R                                                       | n | Yield,<br>percent | M.P., °C.    | Recrystallization<br>solvent | Formula                                           | Calcd. |     |      |      | Found |     |      |      | CHCl <sub>3</sub><br>$\lambda_{\text{max.}}$ | $E \cdot 10^{-3}$ |
|---------------------------------------------------------|---|-------------------|--------------|------------------------------|---------------------------------------------------|--------|-----|------|------|-------|-----|------|------|----------------------------------------------|-------------------|
|                                                         |   |                   |              |                              |                                                   | C      | H   | N    | S    | C     | H   | N    | S    |                                              |                   |
| CH <sub>2</sub> CH <sub>2</sub> CH <sub>3</sub> .....   | 5 | 94                | 212-213 dec. | Ethanol.....                 | C <sub>18</sub> H <sub>22</sub> N <sub>2</sub> S  | 72.5   | 7.4 | 9.4  | 10.7 | 72.3  | 7.6 | 9.2  | 10.5 | 243                                          | 9.4               |
| CH <sub>2</sub> CH <sub>2</sub> N <sub>3</sub> O.....   | 5 | 76                | 170-172      | do.....                      | C <sub>21</sub> H <sub>27</sub> N <sub>3</sub> OS | 68.3   | 7.4 | 11.4 | 8.7  | 68.0  | 7.6 | 11.7 | 8.7  | <sup>c</sup> 245                             | 9.5               |
| CH <sub>2</sub> CH <sub>2</sub> OH.....                 | 5 | 94                | 226-227 dec. | Chloroform-<br>ethanol.....  | C <sub>17</sub> H <sub>20</sub> N <sub>2</sub> OS | 68.0   | 6.7 | 9.3  | 10.7 | 67.8  | 7.0 | 9.1  | 10.9 | <sup>b</sup> 353                             | 18.0              |
| CH <sub>2</sub> CH(CH <sub>3</sub> ) <sub>2</sub> ..... | 5 | 78                | 249-250 dec. | Acetonitrile                 | C <sub>19</sub> H <sub>24</sub> N <sub>2</sub> S  | 73.0   | 7.7 | 9.0  | 10.3 | 72.0  | 7.5 | 8.8  | 10.5 | 358                                          | 19.7              |
| CH <sub>2</sub> CH <sub>2</sub> CH <sub>3</sub> .....   | 4 | 86                | 201-202      | Methanol.....                | C <sub>17</sub> H <sub>20</sub> N <sub>2</sub> S  | 71.8   | 7.1 | 9.9  | 11.3 | 71.6  | 6.8 | 9.5  | 10.9 | 348                                          | 21.8              |
| CH <sub>2</sub> CH(CH <sub>3</sub> ) <sub>2</sub> ..... | 4 | 87                | 198-200      | Acetonitrile                 | C <sub>18</sub> H <sub>22</sub> N <sub>2</sub> S  | 72.4   | 7.4 | 9.4  | 10.7 | 72.6  | 7.3 | 9.6  | 10.9 | 354                                          | 22.0              |

TABLE IX.—INTERMEDIATES



| R                                                | n | Yield, percent    | M.P., °C.      | Recrystallization solvent                   | Formula                                           | Calculated |     |     |     | Found |     |     |     | CHCl <sub>3</sub> , λ <sub>max.</sub> | E × 10 <sup>-3</sup> |
|--------------------------------------------------|---|-------------------|----------------|---------------------------------------------|---------------------------------------------------|------------|-----|-----|-----|-------|-----|-----|-----|---------------------------------------|----------------------|
|                                                  |   |                   |                |                                             |                                                   | C          | H   | N   | S   | C     | H   | N   | S   |                                       |                      |
| CH <sub>2</sub> C(CH <sub>3</sub> ) <sub>3</sub> | 5 | 62                | 155-156 dec.   | CH <sub>2</sub> Cl <sub>2</sub><br>ligroin. | C <sub>20</sub> H <sub>25</sub> N <sub>2</sub> OS | 69.7       | 8.2 | 8.1 | 9.3 | 69.4  | 8.1 | 8.0 | 9.5 | { 295<br>407                          | 11.4<br>13.5         |
|                                                  | 5 | 65                | 161-162 dec.   | Same as above.                              | C <sub>21</sub> H <sub>26</sub> N <sub>2</sub> OS | 70.8       | 7.9 | 7.9 | 9.0 | 70.5  | 7.6 | 7.6 | 8.9 | { 292<br>403                          | 12.9<br>15.6         |
| CH <sub>2</sub> C(CH <sub>3</sub> ) <sub>3</sub> | 4 | 88                | 165-166 dec.   | do                                          | C <sub>19</sub> H <sub>24</sub> N <sub>2</sub> OS | 69.1       | 7.9 | 8.5 | 9.7 | 68.9  | 7.8 | 8.6 | 9.9 | { 298<br>406                          | 10.2<br>13.0         |
|                                                  | 4 | 90                | 161-162.5 dec. | do                                          | C <sub>20</sub> H <sub>25</sub> N <sub>2</sub> OS | 70.1       | 7.7 | 8.2 | 9.4 | 70.1  | 8.0 | 7.8 | 9.1 | { 287<br>401                          | 12.2<br>15.7         |
| CH(CH <sub>3</sub> ) <sub>2</sub>                | 5 | 65 ± 138-140 dec. |                |                                             | C <sub>19</sub> H <sub>24</sub> N <sub>2</sub> OS |            |     |     |     |       |     |     |     | { 290<br>402                          | 12.0<br>16.3         |

<sup>1</sup> Crude.

TABLE X



4(1H)-pyrimidinemethione compounds

| R                                                | n | Yield, percent | M.P., °C.    | Recrystallization solvent | Formula                                           | Calculated |     |     |      | Found |     |     |      | CHCl <sub>3</sub> max. | E × 10 <sup>-3</sup> |
|--------------------------------------------------|---|----------------|--------------|---------------------------|---------------------------------------------------|------------|-----|-----|------|-------|-----|-----|------|------------------------|----------------------|
|                                                  |   |                |              |                           |                                                   | C          | H   | N   | S    | C     | H   | N   | S    |                        |                      |
| CH <sub>2</sub> C(CH <sub>3</sub> ) <sub>3</sub> | 5 | 93             | 221-222      | Acetonitrile              | C <sub>20</sub> H <sub>25</sub> N <sub>2</sub> S  | 73.5       | 8.0 | 8.6 | 9.8  | 73.6  | 8.3 | 8.4 | 9.7  | { 270<br>367           | 10.8<br>18.3         |
|                                                  | 5 | 92             | 241-242 dec. | Ethanol                   | C <sub>21</sub> H <sub>26</sub> N <sub>2</sub> OS | 74.5       | 7.7 | 8.3 | 9.5  | 74.6  | 7.5 | 8.3 | 9.4  |                        |                      |
| CH <sub>2</sub> C(CH <sub>3</sub> ) <sub>3</sub> | 4 | 95             | 216-217.5    | Acetonitrile              | C <sub>19</sub> H <sub>24</sub> N <sub>2</sub> S  | 73.0       | 7.7 | 9.0 | 10.3 | 72.7  | 7.8 | 8.8 | 10.4 | { 270<br>361           | 10.7<br>20.8         |
|                                                  | 4 | 81             | 235-236 dec. | Ethanol                   | C <sub>20</sub> H <sub>25</sub> N <sub>2</sub> S  | 74.0       | 7.5 | 8.6 | 9.9  | 74.0  | 7.3 | 8.6 | 9.8  |                        |                      |

The advantage of using mild reaction conditions is illustrated by the following chart:



The term "hindered amine" as used herein refers, for example, to a primary organic amine which is branched at the 1-position and reacts with difficulty. Isopropylamine, secondary butylamine, tertiary butylamine and cyclohexylamine, disclosed herein, are hindered amines of the character just defined. Neopentylamine is also a hindered amine. Broadly the term "hindered amine" as used herein covers primary amines which undergo reaction with difficulty because of steric hindrance. Steric hindrance is believed to be the reason why amines, otherwise suitable (sufficiently basic, etc.) react with difficulty. Aniline, for example, is not a hindered amine as this term is used herein.

The effectiveness of the 4-pyrimidinethiones in reducing fog according to the invention is shown in the following examples summarized in Table IV. In the examples, samples of the compounds listed were added to separate portions of a high

silver bromoiodide emulsion which has been panchromatically sensitized with a cyanine dye. Each emulsion sample was coated on a cellulose acetate film support at a coverage of 459 mg. of silver and 1040 mg. of gelatin per square foot. A sample of each film coating was exposed on an Eastman 1B sensitometer, processed for 5 minutes in Kodak DK-50 developer, fixed, washed and dried. The results reported are in relation to control.

TABLE IV

| Compound of Example No. | Conc. g./mole of silver | Fresh test     |          |     | One week incubation test |          |      | 15 |
|-------------------------|-------------------------|----------------|----------|-----|--------------------------|----------|------|----|
|                         |                         | Relative speed | $\gamma$ | Fog | Relative speed           | $\gamma$ | Fog  |    |
| Control.....            | .....                   | 100            | 1.53     | .16 | 54                       | 1.09     | .49  |    |
| 5.....                  | .09                     | 85             | 1.38     | .17 | 68                       | 1.18     | .22  |    |
| 6.....                  | .09                     | 71             | 1.23     | .20 | 59                       | 1.00     | .22  |    |
| 4.....                  | .09                     | 59             | 1.18     | .16 | 33                       | 1.08     | .24  |    |
| 1.....                  | .03                     | 95             | 1.38     | .15 | 83                       | 1.25     | .18  |    |
| 12.....                 | .03                     | 82             | 1.45     | .16 | 45                       | 1.22     | .37  |    |
| 2.....                  | .03                     | 69             | 1.35     | .19 | 40                       | 1.20     | .43  |    |
| Control.....            | .....                   | 100            | 1.53     | .22 | 36                       | .83      | 1.08 |    |
| 10.....                 | .16                     | 80             | 1.23     | .26 | 57                       | 1.08     | .35  |    |
| 11.....                 | .03                     | 85             | 1.48     | .21 | 59                       | 1.07     | .50  |    |
| Control.....            | .....                   | 100            | 1.43     | .15 | 63                       | 1.13     | .38  |    |
| 15.....                 | .0009                   | 91             | 1.25     | .14 | 68                       | 1.15     | .33  |    |
| 16.....                 | .0009                   | 100            | 1.37     | .14 | 71                       | 1.18     | .32  |    |
| 17.....                 | .0009                   | 97             | 1.33     | .13 | 65                       | 1.10     | .32  |    |

The preparation of photographic silver halide emulsions such as are suitably stabilized with the 4-pyrimidinethiones of the invention typically involves three separate operations:

1. emulsification and digestion of silver halide,
2. the freeing of the emulsion of excess water-soluble salts, suitably by washing with water, and
3. the second digestion or 'after-ripening' to obtain increased emulsion speed or sensitivity. (Mees, "The Theory of the Photographic Process," 1954). The new antifoggants can be added to the emulsion before the final digestion or after-ripening or it can be added immediately prior to the coating.

The silver halide emulsion or photographic element containing the antifoggants of this invention can contain conventional addenda such as gelatin plasticizers, coating aids, and hardeners such as aldehyde hardeners, e.g., formaldehyde, mucochloric acid, glutaraldehyde bis(sodium bisulfite), maleic dialdehyde, aziridines, dioxane derivatives and oxypolysaccharides. Spectral sensitizers which can be used are the cyanines, merocyanines, complex (trinuclear) cyanines, complex (trinuclear) merocyanines, styryls, and hemicyanines. Sensitizing dyes useful in sensitizing such emulsions are described, for example, in U.S. Pat. Nos. 2,526,632 Brooker and White, issued Oct. 24, 1950, and 2,503,776 of Sprague, issued Apr. 11, 1950. Developing agents can also be incorporated into the silver halide emulsion if desired or can be contained in a contiguous layer. Various silver salts can be used as the sensitive salt such as silver bromide, silver iodide, silver chloride, or mixed silver halides such as silver chlorobromide or silver bromoiodide. The silver halides used can be those which form latent images predominantly on the surface of the silver halide grains or those which form latent images inside the silver halide crystals such as described in U.S. Pat. No. 2,592,250 of Davey and Knott issued Apr. 8, 1952.

The silver halide emulsion layer of a photographic element containing the antifoggants of the invention can contain any of the hydrophilic, water-permeable binding materials suitable for this purpose. Suitable materials include gelatin, colloidal albumin, polyvinyl compounds, cellulose derivatives, acrylamide polymers, etc. Mixtures of these binding agents can also be used. The binding agents for the emulsion layer of the photographic element can also contain dispersed polymerized vinyl compounds. Such compounds are disclosed, for example, in U.S. Pat. Nos. 3,142,568 of Nottorf, issued July 28, 1964; 3,193,386 of White, issued July 6, 1965; 3,062,674 of Houck, Smith and Yudelson, issued Nov. 6, 1962; and

3,220,844 of Houck, Smith and Yudelson, issued Nov. 30, 1965; and include the water-insoluble polymers of alkyl acrylates and methacrylates, acrylic acid, sulfoalkyl acrylates or methacrylates and the like.

5 The silver halide emulsion of a photographic element containing the antifoggants of the invention can be coated on a wide variety of supports. Typical supports are cellulose nitrate film, cellulose ester film, polyvinyl acetal film, polystyrene film, poly(ethylene terephthalate) film and related films or 10 resinous materials as well as glass, paper, metal and the like. Supports such as paper which are coated with  $\alpha$ -olefin polymers, particularly polymers of  $\alpha$ -olefins containing two or more carbon atoms, as exemplified by polyethylene, polypropylene, ethylene-butene copolymers and the like can also be employed.

The speed of the photographic emulsions containing the antifoggants of the invention can be further enhanced by including in the emulsions a variety of hydrophilic colloids such as carboxymethyl protein of the type described in U.S. Pat. No. 3,011,890 of Gates, Jr., Miller and Koller, issued Dec. 5, 1961, and polysaccharides of the type described in Canadian Pat. No. 635,206 of Koller and Russell issued Jan. 23, 1962.

Photographic emulsions containing the antifoggants of the invention can also contain speed-increasing compounds such as quaternary ammonium compounds, polyethylene glycol or thioethers. Frequently, useful effects can be obtained by adding the aforementioned speed-increasing compounds to the photographic developer solutions instead of, or in addition to, the photographic emulsions.

30 Photographic elements containing the antifoggants of the instant invention can be used in various kinds of photographic systems. In addition to being useful in X-ray and other nonoptically sensitized systems, they can also be used in orthochromatic, panchromatic and infrared sensitive systems. The sensitizing addenda can be added to photographic systems before or after any sensitizing dyes which are used.

Photographic emulsions containing the antifoggants of the invention can be used in color photography, for example, 40 emulsions containing color-forming couplers or emulsions to be developed by solutions containing couplers or other color-generating materials, emulsions of the mixed-packet type such as described in U.S. Pat. No. 2,698,794 of Godowsky, issued Jan. 4, 1955; in silver dye-bleach systems; and emulsions of 45 the mixed-grain type such as described in U.S. Pat. No. 2,592,243 of Carroll and Hanson, issued Apr. 8, 1952.

Silver halide emulsions containing the antifoggants of the invention can be sensitized using any of the well-known 50 techniques in emulsion making, for example, by digesting with naturally active gelatin or various sulfur, selenium, tellurium compounds and/or gold compounds. The emulsions can also be sensitized with salts of noble metals of Group VIII of the Periodic Table which have an atomic weight greater than 100.

55 Silver halide emulsions containing the antifoggants of the invention can be used in diffusion transfer processes which utilize the undeveloped silver halide in nonimage areas of the negative to form a positive by dissolving the undeveloped silver halide and precipitating it on a silver layer in close proximity to the original silver halide emulsion layer. Such processes are described in U.S. Pat. Nos. 2,352,014 of Rott, issued June 20, 1944; 2,543,181 of Land, issued Feb. 27, 1951; and 3,020,155 of Yackel, Yutzy, Foster and Rasch, issued Feb. 6, 1962. The emulsions can also be used in diffusion 60 transfer color processes which utilize a diffusion transfer of an imagewise distribution of developer, coupler, or dye, from a light-sensitive layer to a second layer, while the two layers are in close proximity to one another. Silver halide emulsions containing the antifoggants of the invention can be processed in stabilization processes such as the ones described in U.S. Pat. No. 2,614,927 of Broughton and Woodward, issued Oct. 21, 1952, and as described in the article "Stabilization Processing of Films and Papers" by H. D. Russell E. C. Yackel and J. S. Bruce in P.S.A. Journal, Photographic Science and

The antifogging agents of this invention can be incorporated to advantage during manufacture in silver halide emulsions representing the variations described above. Moreover, fog control in binderless silver halide films prepared by vapor deposition of silver halide on a suitable support can be achieved by coating the antifogging agents of the invention over the vapor deposited layer of silver halide.

Combinations of all the above-mentioned addenda can be used if desired.

The amount of antifogging agent can vary quite widely and, in general, will be less than 1 g. per mole of silver. A greater amount can be effectively used where the antifogging agent is incorporated in a layer other than the silver halide emulsion layer, and a lesser amount, generally less than 0.5 g. per mole of silver, and preferably less than 0.1 g. per mole of silver, can be used in the silver halide emulsion layer. The minimum amount is not critical since no adverse effect is incurred by using small amounts. However, it is preferred to use at least 0.0001 g. per mole of silver to obtain a suitable level of fog reduction.

The invention has been described in detail with particular reference to preferred embodiments thereof, but it will be understood that variations and modifications can be effected within the spirit and scope of the invention as described hereinbefore and as defined in the appended claims.

I claim:

1. A light-sensitive photographic silver halide emulsion containing silver halide and a compound selected from the 4-pyrimidinethione compounds having the formula:



wherein R represents hydrogen, an alkyl group having one to 12 carbon atoms, a hydroxyalkyl group having two to six carbon atoms, an alkoxyalkyl group having three to eight carbon atoms, a carboxyalkyl group having two to seven carbon atoms, a  $-(CH_2)_n-COO$  (alkyl having one to four carbon atoms) group, a  $-(CH_2)_n-N$  (alkyl having one to four carbon atoms)<sub>2</sub> group, an aralkyl group, phenyl, tolyl, ethylphenyl, alkoxyphenyl, chlorophenyl, bromophenyl, hydroxyphenyl, xylol, 4-biphenyl, 4-(alkyl) having one to four carbon atoms) morpholino, 1-ethylpyrrolidinyl, 1-ethyl-2-methylpyrrolidinyl, 1-ethylpiperidinyl, n represents an integer from 1 to 4, R<sub>1</sub> represents an alkyl group, an aralkyl group or a benzene nucleus, R<sub>2</sub> represents hydrogen, lower alkyl, lower alkoxy, carb(lower alkoxy) or a benzene nucleus, R<sub>3</sub> represents hydrogen or lower alkyl, wherein R<sub>2</sub> and R<sub>3</sub>, collectively, may represent a polymethylene chain having at least two carbon atoms as an antifogging agent, and wherein the amount of antifogging agent present ranges from at least 0.0001 gram to about 1 gram per mole of silver present in the silver halide emulsion.

2. A light-sensitive photographic silver halide emulsion in accordance with claim 1 wherein R<sub>2</sub> and R<sub>3</sub>, collectively, may represent trimethylene, tetramethylene or pentamethylene.

3. A light-sensitive photographic silver halide emulsion in accordance with claim 1 wherein R<sub>1</sub> is phenyl and wherein R<sub>2</sub> and R<sub>3</sub>, collectively, may represent trimethylene, tetramethylene or pentamethylene.

4. A light-sensitive photographic silver halide emulsion in accordance with claim 1 containing silver halide and a compound selected from the 4-pyrimidinethione compounds having the formula:



wherein R (including n) is defined as in claim 1 as an antifogging agent, and wherein the amount of antifogging agent present ranges from at least 0.0001 gram to about 1 gram per mole of silver present in the silver halide emulsion.

5. A light-sensitive photographic silver halide emulsion in accordance with claim 1 containing silver halide and a compound selected from the 4-pyrimidinethione compounds having the formula:



wherein R (including n) is defined as in claim 1, R<sub>1</sub> represents a lower alkyl group, an aralkyl group or a benzene nucleus as an antifogging agent, and wherein the amount of antifogging agent present ranges from at least 0.0001 gram to about 1 gram per mole of silver present in the silver halide emulsion.

6. A light-sensitive photographic silver halide emulsion in accordance with claim 5 wherein R<sub>1</sub> is phenyl.

7. A light-sensitive photographic silver halide emulsion in accordance with claim 1 containing silver halide and a compound selected from the 4-pyrimidinethione compounds having the formula:



wherein R (including n) is defined as in claim 1 as an antifogging agent, and wherein the amount of antifogging agent present ranges from at least 0.0001 gram to about 1 gram per mole of silver present in the silver halide emulsion.

8. A light-sensitive photographic silver halide emulsion in accordance with claim 7 wherein R represents a lower alkyl group.

9. A light-sensitive photographic silver halide emulsion in accordance with claim 1 containing silver halide and a compound selected from the 4-pyrimidinethione compounds having the formula:



wherein R (including n) is defined as in claim 1 as an antifogging agent, and wherein the amount of antifogging agent present ranges from at least 0.0001 gram to about 1 gram per mole of silver present in the silver halide emulsion.

10. A light-sensitive photographic silver halide emulsion in accordance with claim 9 wherein R represents a lower alkyl group.

11. A light-sensitive photographic silver halide emulsion in accordance with claim 1 containing silver halide and 6,7-dihydro-2-methyl-5H-cyclopentapyrimidine-4(3H)-thione as an antifogging agent.

12. A light-sensitive photographic silver halide emulsion in accordance with claim 1 containing silver halide and 6,7-dihydro-2-phenyl-5H-cyclopentapyrimidine-4(1H)-thione as an antifogging agent.

19

13. A light-sensitive photographic silver halide emulsion in accordance with claim 1 containing silver halide and 6,7-dihydro-1-methyl-2-phenyl-5H-cyclopentapyrimidinethione 4(1H)-thione as an antifoggant.

14. A light-sensitive photographic silver halide emulsion in accordance with claim 1 containing silver halide and 2,5-diphenyl-1-(2-hydroxyethyl)-4(1H)-pyrimidinethione as an antifoggant.

15. A light-sensitive photographic silver halide emulsion in accordance with claim 1 containing silver halide and 2,5-diphenyl-1-methyl-4(1H)-pyrimidinethione as an antifoggant.

16. A photographic element comprising a support having

20

thereon a layer containing a light-sensitive emulsion of claim 1.

17. A photographic element comprising a support having thereon a layer containing a light-sensitive emulsion of claim 2.

18. A photographic element comprising a support having thereon a layer containing a light-sensitive emulsion of claim 5.

19. A photographic element comprising a support having thereon a layer containing a light-sensitive emulsion of claim 11.

\* \* \* \* \*

15

20

25

30

35

40

45

50

55

60

65

70

75

UNITED STATES PATENT OFFICE  
CERTIFICATE OF CORRECTIONPatent No. 3,615,621 Dated October 26, 1971Inventor(s) Robert W. Lamon

It is certified that error appears in the above-identified patent and that said Letters Patent are hereby corrected as shown below:

Col. 2, line 32, "R<sub>13</sub>" should be ---R<sub>3</sub>---.

Col. 1, line 62, "(-CH<sub>2</sub>CH<sub>2</sub>CH<sup>2</sup>CH<sub>2</sub>CH<sub>2</sub>=)" should be  
---(-CH<sub>2</sub>CH<sub>2</sub>CH<sub>2</sub>CH<sub>2</sub>CH<sub>2</sub>-)---.

Col. 5, line 27, delete "4".

Col. 5, between lines 27 and 28, insert ---Example 4--- centered.

Col. 6, line 32, "6,7,9,9" should read ---6,7,8,9---.

Col. 6, line 34, insert ---Benzoyl--- before "isothiocyanate".

Col. 6, line 49, "( 2100)" should be ---( 21000)---.

Col. 8, line 46, after "cycloheptene" insert ---having the formula---.

Col. 9, line 3, " phenylbenzoxamine" should be ---phenylbenzoxazine---.

Table IV, first structure should be



UNITED STATES PATENT OFFICE  
CERTIFICATE OF CORRECTION

Patent No. 3,615,621

Dated October 26, 1971

Inventor(s) Robert W. Lamon

It is certified that error appears in the above-identified patent and that said Letters Patent are hereby corrected as shown below:

Page 2

Table V, last line under heading "Found C", "60.6" should be ---60.0---.

Table VI, line 5, "a<sub>69</sub>" should be ---<sup>b</sup>69---.

Table VII, line 5, under heading "Calculated H", "6.1" should be ---6.7---.

Col. 11, line 54, after "4(1H)" insert ---pyrimidinethione---.

Col. 12, line 51, "4(1H-thione" should be ---4(1H)-thione---.

Table VIII, structure should be



Table VIII, heading "EX10<sup>-</sup>" should be ---E X 10<sup>-3</sup>---.

Table X, heading "EX10<sup>-</sup><sub>3</sub>" should be ---E X 10<sup>-3</sup>---.

UNITED STATES PATENT OFFICE  
CERTIFICATE OF CORRECTION

Patent No. 3,615,621 Dated October 26, 1971

Inventor(s) Robert W. Lamon

It is certified that error appears in the above-identified patent and that said Letters Patent are hereby corrected as shown below:

Page 3

Table X, structure should be



Col. 13, first structure on left should be



Col. 19, line 3, "cyclopentapyrimidinethione" should be  
---cyclopentapyrimidine---.

Signed and sealed this 5th day of December 1972.

(SEAL)

Attest:

EDWARD M.FLETCHER, JR.  
Attesting Officer

ROBERT GOTTSCHALK  
Commissioner of Patents